

April 8, 1941.

F. G. WAHL

2,237,535

METHOD OF MAKING WELDED CONNECTIONS FOR SHEET METAL ARTICLES

Filed Dec. 9, 1938

Fig. 1.



Fig. 2.



Fig. 5.



Fig. 9.

INVENTOR.  
Fred G. Wahl

Barnes, Kuelle, Laughlin & Rauch  
ATTORNEYS

## UNITED STATES PATENT OFFICE

2,237,535

## METHOD OF MAKING WELDED CONNECTIONS FOR SHEET METAL ARTICLES

Frederick G. Wahl, Detroit, Mich., assignor of one-half to Gordon M. Evans, Detroit, Mich.

Application December 9, 1938, Serial No. 244,813

3 Claims. (Cl. 113—120)

This invention relates to the making of articles from sheet metal or the like wherein two or more pieces are joined together at a seam and particularly where the article thus formed is to be finished with a surface of porcelain or the like.

The invention can be disclosed and described in connection with the making of relatively deep receptacles, such as for example, the tub portion of a washing machine, although, of course, the invention is not limited to such an article. It has been the practice to make the tub of a washing machine from a single piece of metal subjected to a drawing operation, and then the shaped article, in many cases, is given an application of porcelain. There is a considerable draw in the metal in this case and fairly thick sheet stock has to be employed to stand the draw. Also, the drawing machinery is expensive and large, with the result that there is a considerable outlay for equipment.

This invention aims to provide a method wherein an article such as a deep receptacle can be made from two or more pieces of sheet metal without any substantial drawing action. Thus lighter stock can be used and the initial capital expenditure for equipment is materially reduced and, moreover, very little sheet metal is wasted in the process. To these ends sheet metal parts may be suitably fashioned by a rolling or forming operation or by a stamping operation, or both, and parts to be united are provided with flanges arranged to abut each other. These flanges are then welded together, but where the flanges meet, a groove or crack is formed, and this will not properly take a surface finish of porcelain or the like. To overcome this, the metal of the parts is worked with a spreading action to open up the crack or groove and flatten it out, as far as the weld will permit. This minimizes the dimensions of the crack or groove to such an extent that a finish of porcelain or the like can be satisfactorily applied.

In the accompanying drawing:

Fig. 1 is a perspective view of a sheet of metal fashioned into cylindrical form with the edges welded together.

Fig. 2 is a cross sectional view of the cylinder with its ends fashioned properly to constitute an upper end and flange means for attachment to the bottom.

Fig. 3 is an enlarged sectional view taken through the flange illustrated in Fig. 2 and showing welding electrodes.

Fig. 4 is a further enlarged sectional view showing the welded seam.

Fig. 5 is a view enlarged to the size of Fig. 3 illustrating a working operation or spreading operation.

Fig. 6 is a view enlarged to the size of Fig. 4 showing the seam structure after the spreading operation.

Fig. 7 is a diagrammatic view illustrating a finishing operation.

Fig. 8 is an enlarged view showing the surface finish of porcelain or the like.

Fig. 9 is a view similar to Fig. 5 showing a modified arrangement.

15 The vessel or tub may be fashioned from a sheet of metal such as steel fashioned into cylindrical form with the edges butt welded together. The cylindrical form is shown in Fig. 1, and the cylindrical form 1 becomes the side walls of the receptacle. The butt weld at the edges is suitably trimmed and finished. Due to the fact that sheet stock is rolled into cylindrical form relatively light gauge stock may be used. The cylindrical form may next be subjected to a suitable forming operation to fashion the upper edge in the proper manner, as for example, in the form of an inwardly extending roll 2. The opposite end may be fashioned with an inwardly extending portion or a suitable radius as illustrated at 3, and the extreme end is formed with an outwardly projecting flange 4.

The bottom of the receptacle may be a sheet metal stamping 5 which may also be of relatively light gauge stock due to the fact that the stamping is so shallow, and the bottom is provided with a flange 6 arranged to abut against the flange 4 as illustrated. The flanges 4 and 6 are properly located relative to each other and are to be welded together. Prior to the complete welding operation, however, the flanges may be tacked or temporarily connected by spaced welds. The bottom 5 preferably has its outer zone on a radius to somewhat match the radius 3 of the body.

45 The next step in the making of the receptacle is that of welding the flanges 4 and 6, and this may be done by opposed roller electrodes 7 and 8. The receptacle may be revolved on its axis with the flanges moving between the electrodes to form a continuous fluid tight weld entirely around the vessel. This weld is indicated by the overhatch 9 in the enlarged Fig. 4. However, it will be noted that quite a substantial groove or crack is left on the interior of the vessel, as indicated at 10. This cannot be properly finished

with porcelain or the like, as the porcelain cracks or separates in this groove and may leave some exposed metal. Moreover, the groove can be seen with the naked eye which is objectionable, and it is not a sanitary arrangement in a thing such as a tub for a washing machine.

Accordingly, the metal is now worked or spread to minimize the dimensions of this groove. This may be done after the manner illustrated in Fig. 5. The apparatus used for this purpose is subject to variation insofar as this invention is concerned, but one way of accomplishing this spreading action is to use a roller 15 disposed to engage the metal on the inside of the seam and a roller 16 arranged to engage the metal on the outside and having a groove 17 for the reception of the flange constituted by the overlapping parts 4 and 6. The flange, however, does not seat in the bottom of the groove 17, with the result that the vessel and the rollers are more or less in a floating position relative to each other. The rollers 15 and 16 are urged toward each other with pressure, and a relative rotary motion is caused between the vessel and the rollers. In this action the metal of both the shell 1 and the bottom 5 on opposite sides of the seam is worked and spread apart. This spreading action will continue until the metal spreads to the point where the weld prevents further spreading. In other words, as Fig. 4 is viewed, the metal portions on opposite sides of the groove are spread outwardly away from each other, and more or less flattened. The weld line in Fig. 4 is indicated at X; by weld lines we mean the innermost portions of the flanges 4 and 6 which are weld united. The spreading continues and the weld line is caused to shift toward the sides of the receptacle or the metal stock, at which time the weld connection is drawn taut, so to speak, and further spreading stopped. As a result, the inner surfaces of the sheet 1 and sheet 5 come together in a substantially flush manner with the weld connection joining the same and lying substantially at the line Y in Fig. 6.

Now it may well be, and perhaps will be, that the weld line X will vary in its position. In some spots the weld line may be in the position shown in Fig. 4, and in other spots on the same job the weld line may be further outward or towards the ends of the flanges and in still other spots be further inward toward the groove. Due to the floating arrangement of the spreading rollers, there is a little greater spreading action where the weld line is positioned more toward the outer edge of the flange, resulting perhaps in a slight increase in the bulge and the ultimate radius at these spots; where the weld line is closer to the groove the resultant bulge and radius may be less than in other spots. However, these slight variations are not visible to the eye, and there is no resultant objectionable defect.

It will be noted that the crack between the flanges is now minimized and the inner surfaces of the sheets 1 and 2 more or less abut each other smoothly with a weld line therebetween. The receptacle may now be finished by finishing the roll at the upper edge or other suitable or desirable finishing operations and the receptacle is ready to be cleaned or pickled and then given a base coat of porcelain. This is illustrated in Fig. 7 where the material is sprayed on to the shell by a suitable gun 20. As is well known to those versed in the art, the tub may now be baked at a suitable temperature and subsequently a finish coat of porcelain sprayed over the base

coat and then the vessel subjected to another baking operation. The porcelain applies evenly over the surfaces and over the smooth weld line X so that in the finished job no weld on the interior is appreciably visible. In Fig. 8 a more or less diagrammatic illustration is given showing the finished job with the porcelain coating 21.

A variation in the spreading step is illustrated in Fig. 9. The interior roller 15 may be the same as that shown in Fig. 5, but exterior rollers 22 and 23 are applied to the flange with pressure. Relative rotation between the roller assembly and the vessel causes the metal to spread to minimize the dimensions of the crack or groove and result in the structure as shown in Fig. 6.

In the initial fashioning of the flanges on the sheet metal parts, it is desirable to have a considerable radius at the juncture between the sheet metal body and the flange, as this is good practice in sheet metal working, as the metal might be ruptured or sheared if an attempt be made to form a sharp bend or break line. It is due to the opposing curved surfaces formed on the radii that the initial groove is formed. The working and spreading of the metal so reduces the dimensions of the groove that a finish of porcelain or the like may be satisfactorily applied, whereas the finish could not be satisfactorily applied with a groove of the initial dimensions. Furthermore, the provision of initial relatively long radii at the flanges is desirable as such a formation lends itself to the spreading action, and in fact facilitates the spreading process.

In the finished article there is, of course, the projecting exterior flange which may, if desired, be trimmed to reduce its width, but which may be concealed in any suitable way, as for example, by the attachment of the legs for the tub, or the projecting flange may be made more or less ornamental by merely disposing a bead or rubber or the like over it.

It has been found expedient to locate the flanges 4 and 6 at a corner of the vessel. In this way, the adjacent metal takes a direction away from the welding rolls 7 and 8, as shown in Fig. 3, whereby the weld between the flanges 4 and 6 may be taken well inwardly of the flange toward the body of the vessel. However, it is within the invention to locate the flanges in parts which are not angularly disposed relative to each other. Furthermore, by placing the flanges at a corner or the like, especially where there is considerable radius in the ultimate job, as shown in Fig. 7, the bulging effect which may be produced by the spreading is more or less absorbed in the curvature and loses any visible identity. The initial radius given to the body of the vessel at 3 and the initial radius adjacent the edges of the bottom may be somewhat less than that of the ultimate radius. This is shown in an exaggerated manner as will be evidenced by comparison of Figs. 2 and 7. In the spreading and bulging operation, the radii may be slightly increased and the resultant curvature of the adjacent parts of the body and bottom may be substantially the same. The invention is not limited to a porcelain finish, but is applicable to other finishes where a crack or groove is undesirable.

I claim:

1. The method of making a receptacle which comprises fashioning a sheet metal blank into a tubular body having a circumferentially smooth

wall at least adjacent one end, forming a flange at said end of the body with the flange meeting the tubular wall of the body on a curve, fashioning a bottom from sheet metal and forming a flange on the peripheral edge of the bottom with the flange meeting the metal in the bottom on a curve, placing the body and the bottom together with the flanges in abutting relationship with the curved portions defining a groove, welding the interfacial surfaces of the flanges together, working the metal of the body and the bottom adjacent the flanges to cause a spreading action substantially until the weld connection is drawn taut to reduce the dimensions of said groove to such a size as to present a surface for the reception of a finish such as porcelain or the like.

2. The method of making a receptacle which comprises, fashioning a sheet metal blank into a tubular body having a circumferentially smooth wall at least adjacent one end, forming a circumferential outwardly extending flange at said one end of the body with the flange meeting the tubular wall of the body on a curve, fashioning a bottom for the receptacle of sheet metal, forming a circumferential outwardly extending flange thereon which meets the metal of the bottom on

a curve, placing the bottom and the body together with the flanges in abutting relationship, with the curve portions defining a groove, welding the interfacial areas of the flanges together, working the metal at and adjacent the curved portions to cause a spreading action until the weld connection is substantially drawn taut to thereby reduce the dimensions of the groove to such a size as to present a surface for the reception of a finish such as porcelain or the like.

3. The method of uniting two sheet metal parts in a seam adapted to receive a finish such as porcelain or the like which comprises, forming a flange on the edge of one sheet metal part with the flange joining the body of the part on a curve, forming a flange on the other sheet metal part with the flange joining the body of the part on a curve, placing the flanges together in abutting relationship, welding the interfacial surfaces of the flanges together with the curves defining a groove, working the metal in and adjacent the curves to cause a spreading action substantially until the weld connection is drawn taut to thereby reduce the dimensions of the groove to such a size as to receive the said finish.

FRED G. WAHL.